

# United States Patent Office

2,747,978

Patented May 29, 1956

1

2,747,978

## STABILIZED ORGANIC COMPOSITIONS

Katherine Weiss Closson and James Cowan Boag, Detroit, Mich., assignors to Ethyl Corporation, New York, N. Y., a corporation of Delaware

No Drawing. Application July 26, 1952,  
Serial No. 301,166

3 Claims. (Cl. 44—69)

This invention relates to the stabilization of organic materials normally susceptible to deterioration. More particularly, our invention relates to the inhibition of attack by oxygen and the prolongation of the useful life of such materials.

Hydrocarbon fuels for use in internal combustion spark ignition engines may be classified broadly into three categories, according to the type of engine for which they are manufactured and marketed, such as automotive, aircraft and diesel fuels. Although each type of fuel is composed essentially of hydrocarbons, the type and stability characteristics of the individual hydrocarbon types comprising each fuel differ considerably, as do the relative proportions of the various types in each fuel. For example, typical automotive fuels contain straight and branched chain aliphatics, olefins, naphthenes and some aromatics, typical aircraft fuels are particularly low in olefins and typical diesel fuels contain principally saturated hydrocarbons with a smaller proportion of olefins.

During the refining, manufacturing and blending processes, and during subsequent storage and handling operations, it is unavoidable that these fuels or their ingredients, such as cracked blending stocks, or the highly olefinic stocks for reforming and alkylation, are brought into contact with oxygen. The result of such contact is the formation, by oxidation or polymerization or a combination thereof, of gummy materials which interfere with the efficient utilization of said fuels in the engine.

Automotive gasolines are, in general, more susceptible to this type of degradation by oxygen than aircraft fuels, while in recent years the degradation of fuels for use in compression ignition engines has become more significant. The presence of gummy materials in fuels for spark ignition engines causes valve sticking, lowered spark plug efficiency, piston varnish and associated troubles, while such deteriorated fuels, when used in diesel engines, interfere with the operation of the fuel filters and injectors.

Because of the specifications imposed on fuels by the rigid requirements of present day engines, particularly aircraft engines, it is essential that any material capable of protecting such fuels against deterioration be effective in extremely small quantities, on the order of one pound of additive per five thousand gallons of fuel, so that secondary problems do not arise through their use.

Many other materials in extensive use require protection from the adverse effects of contact with oxygen. One such class of materials is the elastomers, both natural and synthetic. Upon absorption of oxygen such elastomers deteriorate prematurely, lose tensile strength and flexibility and become discolored and embrittled. This absorption can occur during manufacturing operations, fabrication, storage or use. While certain materials have been proposed for the protection of such elastomers from the deleterious action of oxygen, many of such protective substances possess the serious disadvantage, particularly with respect to light colored stocks, that the decomposition products are themselves colored and hence interfere with the color fastness of the stocks being protected.

2

Further examples of materials which require protection from the effects of oxygen include mineral oils, lubricating oils, soaps, and diverse synthetic unsaturated organic materials. In general, our invention is useful in protecting those organic substances which, during the process of manufacturing, handling, storage, or use, become exposed to and absorb oxygen with deleterious effects.

It is, therefore, an object of our invention to provide means for protecting such organic substances which deteriorate in or are affected adversely by oxygen. It is a further object of our invention to provide a class of substances which prevents the formation of gummy oxidation and polymerization products of unstable hydrocarbons in contact with oxygen. Another object of our invention is to provide means for stabilizing hydrocarbon fuels for internal combustion spark and compression ignition engines during the manufacturing, handling, and storage of such fuels prior to their use. A further object of our invention is to provide hydrocarbon fuels containing tetraethyllead which do not deteriorate in contact with oxygen with the resultant formation of gum, and which do maintain for long periods the qualities inherent in such finished fuels at the time of manufacture. Likewise, it is an object of our invention to provide means for preventing embrittlement, discoloration, loss of tensile strength, and other harmful effects in elastomers during the milling, compounding, fabricating, storage, handling, and use of such elastomer stocks. A further object of this invention is to provide means for protecting perishable material or synthetic organic materials from the adverse effects of contact with oxygen. Still further objects of our invention will appear from the description of our invention as hereinafter disclosed.

Throughout the history of the development of effective antioxidant compositions, recourse has been made to compounds containing amine or hydroxy substituents on an aromatic nucleus. This can be substantiated by noting examples of the effective antioxidants used commercially to stabilize organic materials normally susceptible to deterioration. One of the earliest known antioxidants was comprised of mixed phenols from cracked wood tar distillates. Other such antioxidant materials containing said substituents include N,N'-di-sec-butyl-p-phenylenediamine, N-n-butyl-p-aminophenol, 2,4-dimethyl-6-tert-butylphenol, hydroquinone, aniline, tannic acid, p-tolylhydroquinone, tert-butylhydroquinone, 4-methyl-2,6-di-tert-butylphenol, 4,6-di-tert-butyl-m-cresol,  $\alpha$ -naphthylamine,  $\beta$ -naphthylamine, N,N'-di-n-butyl-p-phenylenediamine, N,N'-di-isopropyl phenylenediamine, 2,2-methylene-bis-(4-methyl-6-tert-butylphenol), a mixed antioxidant comprising N,N'-di-sec-butyl-p-phenylenediamine and p-sec-butylaminophenol, p-aminohydroxynaphthols, diamino naphthylamines, the condensation product of butyraldehyde-aniline, aldon- $\alpha$ -naphthylamine, phenyl- $\beta$ -naphthylamine, and the like. However, we have made the startling discovery that the above and other objects of our invention can be accomplished by employing sulfur-containing lead carbamates, certain embodiments of which need not contain arylamine or arylhydroxy groups to provide effective antioxidant materials.

In general, the antioxidants of our invention are characterized by the structure



wherein X and X<sub>1</sub> can be the same or different and are selected from oxygen or sulfur; that is, are chalcogens, and wherein each of R<sub>1</sub>, R<sub>2</sub>, R<sub>3</sub>, and R<sub>4</sub> can be the same or different and are selected from hydrogen or organic radicals. In our preferred embodiments such R groups are aliphatic or cycloaliphatic groups.

In naming certain of the embodiments of the sulfur-

containing lead carbamate of our invention, we prefer to utilize the term lead N,N,N',N'-tetraalkyl-dithiocarbamate, although it is recognized that these substances are also known by the term lead dialkyl-dithiocarbamate.

As will hereinafter be indicated, the compounds of our invention concurrently provide both primary antioxidant activity and synergistic effects to antioxidants of the arylamine type. This we believe is the noteworthy discovery inasmuch as, surprisingly, the lead cation of the class of compounds comprising the antioxidants of our invention in some currently unexplainable manner appears to be intrinsically involved in producing the overall antioxidant effectiveness.

The aliphatic radicals of the antioxidants of our invention can be saturated alkyl radicals such as methyl, ethyl, n-propyl, isopropyl, n-butyl, isobutyl, sec-butyl, t-butyl, n-amyl, and the various positional isomers thereof as, for example, 1-methyl-n-butyl, 2-methyl-n-butyl, 3-methyl - n - butyl, 1,1-dimethyl - n - propyl, 1,2-dimethyl - n - propyl, 2,2-dimethyl - n - propyl, and 1-ethyl-n-propyl, and likewise the corresponding straight and branched chain isomers of hexyl, heptyl, octyl, nonyl, decyl, undecyl, dodecyl, tridecyl, tetradecyl, pentadecyl, hexadecyl, heptadecyl, octadecyl, nonadecyl, eicosyl, and the like. In addition, these aliphatic radicals of the antioxidants of our invention may be unsaturated, containing double bonds, such as ethenyl,  $\Delta^1$ -propenyl,  $\Delta^2$ -propenyl, isopropenyl,  $\Delta^1$ -butenyl,  $\Delta^2$ -butenyl,  $\Delta^3$ -butenyl, and the corresponding branched chain isomers thereof as, for example,  $\Delta^1$ -isobut enyl,  $\Delta^2$ -isobut enyl,  $\Delta^1$ -sec-but enyl,  $\Delta^2$ -sec-but enyl, including 1-methylene- $\Delta^2$ -propenyl,  $\Delta^1$ -pentenyl,  $\Delta^2$ -pentenyl,  $\Delta^3$ -pentenyl,  $\Delta^4$ -pentenyl, and the corresponding branched chain isomers thereof,  $\Delta^1$ -hexenyl,  $\Delta^2$ -hexenyl,  $\Delta^3$ -hexenyl,  $\Delta^4$ -hexenyl,  $\Delta^5$ -hexenyl, and the corresponding branched chain isomers thereof, including 3,3-dimethyl- $\Delta^1$ -butenyl; 2,3-dimethyl- $\Delta^1$ -butenyl; 2,3-dimethyl- $\Delta^2$ -butenyl; 2,3-dimethyl- $\Delta^3$ -butenyl; and 1-methyl-1-ethyl- $\Delta^2$ -propenyl; and similarly, the various isomers of heptenyl, octenyl, nonenyl, decenyl, undecenyl, dodecenyl, tridecenyl, tetradecenyl, pentadecenyl, hexadecenyl, heptadecenyl, octadecenyl, nonadecenyl, eicosenyl, and the like.

In addition, the aliphatic radicals can be substituted. For example, when such substituents are aryl, our antioxidants contain aralkyl radicals such as benzyl,  $\alpha$ -phenyl-ethyl,  $\beta$ -phenyl-ethyl,  $\alpha$ -phenyl-n-propyl,  $\beta$ -phenyl-n-propyl,  $\gamma$ -phenyl - n - propyl,  $\alpha$ -phenyl - isopropyl,  $\beta$ -phenyl - isopropyl,  $\alpha$ -phenyl - n - butyl,  $\beta$ -phenyl - n - butyl,  $\gamma$ -phenyl - n - butyl,  $\delta$ -phenyl - n - butyl,  $\alpha$ -phenyl - isobutyl,  $\beta$ -phenyl - isobutyl,  $\gamma$ -phenyl - isobutyl,  $\alpha$ -phenyl - sec - butyl,  $\beta$ -phenyl - sec - butyl,  $\gamma$ -phenyl - sec - butyl,  $\beta$ -phenyl - t - butyl,  $\alpha'$ -naphthyl - methyl,  $\beta'$ -naphthyl - methyl,  $\alpha$ -( $\alpha'$ -naphthyl) - ethyl,  $\alpha$ -( $\beta'$ -naphthyl) - ethyl,  $\beta$ -( $\alpha'$ -naphthyl) - ethyl,  $\alpha$ -( $\beta'$ -naphthyl) - n - propyl,  $\beta$ -( $\alpha'$ -naphthyl) - n - propyl,  $\alpha$ -( $\beta'$ -naphthyl) - n - propyl,  $\beta$ -( $\beta'$ -naphthyl) - n - propyl,  $\gamma$ -( $\alpha'$ -naphthyl) - n - propyl,  $\gamma$ -( $\beta'$ -naphthyl) - n - propyl,  $\alpha$ -( $\alpha'$ -naphthyl) - isopropyl,  $\alpha$ -( $\beta'$ -naphthyl) - iso - propyl,  $\alpha$ -( $\alpha'$ -naphthyl) - n - butyl,  $\alpha$ -( $\beta'$ -naphthyl) - n - butyl,  $\beta$ -( $\alpha'$ -naphthyl) - n - butyl,  $\beta$ -( $\beta'$ -naphthyl) - n - butyl,  $\gamma$ -( $\alpha'$ -naphthyl) - n - butyl,  $\gamma$ -( $\beta'$ -naphthyl) - n - butyl,  $\delta$ -( $\alpha'$ -naphthyl) - n - butyl,  $\delta$ -( $\beta'$ -naphthyl) - n - butyl,  $\alpha$ -( $\alpha'$ -naphthyl) - iso - butyl,  $\alpha$ -( $\beta'$ -naphthyl) - isobutyl,  $\beta$ -( $\alpha'$ -naphthyl) - isobutyl,  $\beta$ -( $\beta'$ -naphthyl) - isobutyl,  $\gamma$ -( $\alpha'$ -naphthyl) - isobutyl,  $\gamma$ -( $\beta'$ -naphthyl) - isobutyl,  $\alpha$ -( $\alpha'$ -naphthyl) - sec - butyl,  $\alpha$ -( $\beta'$ -naphthyl) - sec - butyl,  $\beta$ -( $\alpha'$ -naphthyl) - sec - butyl,  $\beta$ -( $\beta'$ -naphthyl) - sec - butyl,  $\gamma$ -( $\alpha'$ -naphthyl) - sec - butyl,  $\gamma$ -( $\beta'$ -naphthyl) - sec - butyl,  $\beta$ -( $\alpha'$ -naphthyl) - t - butyl,  $\beta$ -( $\beta'$ -naphthyl) - t - butyl, the corresponding  $\alpha'$  and  $\beta'$  naphthyl derivatives of n-amyl and the various positional isomers thereof as, for example, said derivatives of 1-methyl - n - butyl, 2-methyl - n - butyl, 3-methyl -

n - butyl, 1,1-dimethyl - n - propyl, 1,2-dimethyl - n - propyl, 2,2-dimethyl - n - propyl, 1-ethyl - n - propyl, and likewise said derivatives of the corresponding isomers of hexyl, heptyl, octyl, and the like including eicosyl. Other such aralkyl derivatives include the  $\alpha'$ ,  $\beta'$ , and  $\gamma'$  anthryl of alkyl radicals, such as, for example,  $\alpha'$ -anthryl - methyl,  $\alpha$ -( $\beta'$ -anthryl) - ethyl,  $\beta$ -( $\gamma'$ -anthryl) - ethyl,  $\alpha$ -( $\alpha'$ -anthryl) - n - butyl,  $\delta$ -( $\beta'$ -anthryl) - 2 - methyl - n - amyl, and the like, and corresponding alkyl derivatives of phenanthrene, fluorene, acenaphthene, chrysene, pyrene, triphenylene, naphthacene, and the like.

In addition, the aliphatic portion of such aralkyl radicals of the antioxidants of our invention can be unsaturated, containing double bonds such as  $\alpha$ -phenyl-ethenyl,  $\beta$ -phenyl-ethenyl,  $\alpha$ -phenyl- $\Delta^1$ -propenyl,  $\beta$ -phenyl -  $\Delta^1$ -propenyl,  $\gamma$ -phenyl -  $\Delta^1$ -propenyl,  $\alpha$ -phenyl -  $\Delta^2$ -propenyl,  $\beta$ -phenyl -  $\Delta^2$ -propenyl,  $\gamma$ -phenyl -  $\Delta^2$ -propenyl,  $\alpha$ -phenyl - isopropenyl,  $\beta$ -phenyl - isopropenyl,  $\gamma$ -phenyl - isopropenyl, and similarly, the phenyl derivatives of the isomers of butenyl, pentenyl, hexenyl, heptenyl, and the like, up to and including about eicosenyl. Other such arylalkenyls include  $\alpha$ -( $\alpha'$ -naphthyl) - ethenyl,  $\alpha$ -( $\beta'$ -naphthyl) - ethenyl,  $\beta$ -( $\alpha'$ -naphthyl) - ethenyl,  $\beta$ -( $\beta'$ -naphthyl) - ethenyl,  $\alpha$ -( $\alpha'$ -naphthyl) -  $\Delta^1$ -propenyl,  $\beta$ -( $\beta'$ -naphthyl) -  $\Delta^1$ -propenyl,  $\alpha$ -( $\beta'$ -naphthyl) -  $\Delta^1$ -propenyl,  $\beta$ -( $\beta'$ -naphthyl) -  $\Delta^1$ -propenyl,  $\alpha$ -( $\alpha'$ -naphthyl) -  $\Delta^2$ -propenyl,  $\beta$ -( $\beta'$ -naphthyl) -  $\Delta^2$ -propenyl,  $\alpha$ -( $\beta'$ -naphthyl) -  $\Delta^2$ -propenyl,  $\beta$ -( $\beta'$ -naphthyl) -  $\Delta^2$ -propenyl,  $\alpha$ -( $\alpha'$ -naphthyl) -  $\Delta^2$ -propenyl,  $\beta$ -( $\beta'$ -naphthyl) -  $\Delta^2$ -propenyl,  $\alpha$ -( $\alpha'$ -naphthyl) - isopropenyl,  $\beta$ -( $\beta'$ -naphthyl) - isopropenyl,  $\alpha$ -( $\beta'$ -naphthyl) - isopropenyl,  $\beta$ -( $\beta'$ -naphthyl) - isopropenyl, and the like. In addition, such aromatic derivatives of alkenyls include derivatives of phenanthrene, fluorene, acenaphthene, chrysene, pyrene, triphenylene, naphthacene, and the like.

We also can employ as organic radicals in our antioxidants cycloaliphatic groups such as cyclopropyl, cyclobutyl, cycloamyl, cyclohexyl, cycloheptyl, cyclooctyl, cyclononyl, cyclodecyl, cycloundecyl, cyclododecyl, cyclotridecyl, cyclotetradecyl, cyclopentadecyl, cyclohexadecyl, cycloheptadecyl, cyclooctadecyl, cyclonondecyl, cyclooctadecyl, and such cycloaliphatic radicals as  $\alpha$ -cyclopropyl-ethyl,  $\beta$ -cyclopropyl-ethyl,  $\alpha$ -cyclobutyl-propyl,  $\beta$ -cyclobutyl-propyl,  $\gamma$ -cyclobutyl-propyl,  $\alpha$ -cycloamyl-isopropyl,  $\beta$ -cycloamyl-isopropyl, and the like. Similarly, the cycloaliphatic groups comprise the cycloalkenyls such as  $\alpha$ -cyclohexyl-ethenyl,  $\beta$ -cyclohexyl-ethenyl,  $\alpha$ -cycloheptyl- $\Delta^1$ -propenyl,  $\beta$ -cycloheptyl- $\Delta^1$ -propenyl,  $\alpha$ -cycloheptyl- $\Delta^2$ -propenyl,  $\beta$ -cycloheptyl- $\Delta^2$ -propenyl,  $\alpha$ -cyclooctyl- $\Delta^1$ -propenyl,  $\beta$ -cyclooctyl- $\Delta^1$ -propenyl,  $\alpha$ -cyclooctyl- $\Delta^2$ -propenyl,  $\beta$ -cyclooctyl- $\Delta^2$ -propenyl,  $\alpha$ -cyclooctyl- $\Delta^3$ -propenyl,  $\beta$ -cyclooctyl- $\Delta^3$ -propenyl,  $\alpha$ -cyclooctyl- $\Delta^4$ -propenyl,  $\beta$ -cyclooctyl- $\Delta^4$ -propenyl, and the like.

Thus, the organic radicals of our compounds contain from about 1 to 20 carbon atoms, are saturated or unsaturated, cyclic or acyclic, and the aforementioned can be substituted with at least one aryl group.

When each of X and X<sub>1</sub> of the aforementioned generic structure is sulfur, there is provided a general class of lead dithiocarbamates. Therefore, specific examples of these compounds comprising preferred antioxidants of our invention include lead dithiocarbamate; lead N,N,N',N'-tetraethyl dithiocarbamate; lead N,N,N',N'-tetraethyl dithiocarbamate; lead N,N,N',N'-tetraisopropyl dithiocarbamate; lead N,N,N',N'-tetra-n-butyl dithiocarbamate; lead N,N,N',N'-tetraisobutyl dithiocarbamate; lead N,N,N',N'-tetra-sec-butyl dithiocarbamate; lead N,N,N',N'-tetra-t-butyl dithiocarbamate; lead N,N,N',N'-tetra-n-amyl dithiocarbamate; lead N,N,N',N'-tetra-(1-methyl-n-butyl)-dithiocarbamate; lead N,N,N',N'-tetra-(2-methyl-n-butyl)-dithiocarbamate; lead N,N,N',N'-tetra-(3-methyl-n-butyl)-dithiocarbamate; lead N,N,N',N'-tetra-(1,1-dimethyl-n-propyl)-dithiocarbamate; lead N,N,N',N'-tetra-(1,2-dimethyl-n-propyl)-

dithiocarbamate; lead N,N,N',N'-tetra-(2,2-dimethyl-n-propyl)-dithiocarbamate; lead N,N,N',N'-tetra-(1-ethyl-n-propyl)-dithiocarbamate; and the like.

Similarly, our dithiocarbamate antioxidants comprise alkenyl substituted compounds providing, for example, such compounds as lead N,N,N',N'-tetraethenyl dithiocarbamate; lead N,N,N',N'-tetra-( $\Delta^1$ -propenyl) dithiocarbamate; lead N,N,N',N'-tetra-( $\Delta^2$ -propenyl) dithiocarbamate; lead N,N,N',N'-tetra-( $\Delta^1$ -isopropenyl) dithiocarbamate; lead N,N,N',N'-tetra-( $\Delta^1$ -butenyl) dithiocarbamate; lead N,N,N',N'-tetra-( $\Delta^2$ -butenyl) dithiocarbamate; lead N,N,N',N'-tetra-( $\Delta^3$ -butenyl) dithiocarbamate; lead N,N,N',N'-tetra-( $\Delta^1$ -isobut enyl) dithiocarbamate; lead N,N,N',N'-tetra-( $\Delta^2$ -isobut enyl) dithiocarbamate; lead N,N,N',N'-tetra-( $\Delta^1$ -sec-but enyl) dithiocarbamate; lead N,N,N',N'-tetra-( $\Delta^2$ -sec-but enyl) dithiocarbamate; and the like, including related compounds as, for example, lead N,N,N',N'-tetra-(1-methylene- $\Delta^2$ -propenyl) dithiocarbamate.

Furthermore, our dithiocarbamate antioxidants comprise aralkyl substituted compounds providing, for example, such compounds as lead N,N,N',N'-tetra-( $\alpha$ -phenyl-ethyl) dithiocarbamate; lead N,N,N',N'-tetra-( $\beta$ -phenylethyl) dithiocarbamate; lead N,N,N',N'-tetra-( $\alpha$ -phenyl-n-propyl) dithiocarbamate; lead N,N,N',N'-tetra-( $\beta$ -phenyl-n-propyl) dithiocarbamate; lead N,N,N',N'-tetra-( $\gamma$ -phenyl-n-propyl) dithiocarbamate; lead N,N,N',N'-tetra-( $\alpha$ -phenylisopropyl) dithiocarbamate; lead N,N,N',N'-tetra-( $\beta$ -phenylisopropyl) dithiocarbamate; lead N,N,N',N'-tetra-( $\alpha$ -( $\alpha'$ -naphthyl)-n-butyl) dithiocarbamate; lead N,N,N',N'-tetra-( $\alpha$ -( $\beta'$ -naphthyl)-n-butyl) dithiocarbamate; lead N,N,N',N'-tetra-( $\beta$ -( $\alpha'$ -naphthyl)-n-butyl) dithiocarbamate; lead N,N,N',N'-tetra-( $\beta$ -( $\beta'$ -naphthyl)-n-butyl) dithiocarbamate; lead N,N,N',N'-tetra-( $\alpha$ -( $\alpha'$ -tetrahydronaphthyl)-isoamyl) dithiocarbamate; lead N,N,N',N'-tetra-( $\beta$ -( $\alpha'$ -tetrahydronaphthyl)-isoamyl) dithiocarbamate; lead N,N,N',N'-tetra-( $\gamma$ -( $\alpha'$ -tetrahydronaphthyl)-isoamyl) dithiocarbamate; lead N,N,N',N'-tetra-( $\delta$ -( $\alpha'$ -tetrahydronaphthyl)-isoamyl) dithiocarbamate; lead N,N,N',N'-tetra-( $\alpha$ -( $\alpha'$ -tetrahydronaphthyl)-isoamyl) dithiocarbamate; lead N,N,N',N'-tetra-( $\beta$ -( $\beta'$ -tetrahydronaphthyl)-isoamyl) dithiocarbamate; lead N,N,N',N'-tetra-( $\gamma$ -( $\beta'$ -tetrahydronaphthyl)-isoamyl) dithiocarbamate; lead N,N,N',N'-tetra-( $\delta$ -( $\beta'$ -tetrahydronaphthyl)-isoamyl) dithiocarbamate; and the like. Similarly, our dithiocarbamate antioxidants comprise aralkenyl substituted compounds providing, for example, such compounds as lead N,N,N',N'-tetra-( $\alpha$ -( $\alpha'$ -anthryl)- $\Delta^1$ -n-pentenyl) dithiocarbamate; lead N,N,N',N'-tetra-( $\alpha$ -( $\beta'$ -anthryl)- $\Delta^2$ -n-pentenyl) dithiocarbamate; lead N,N,N',N'-tetra-( $\alpha$ -( $\gamma'$ -anthryl)- $\Delta^3$ -n-pentenyl) dithiocarbamate; lead N,N,N',N'-tetra-( $\beta$ -( $\alpha$ -phenanthryl)- $\Delta^1$ -n-pentenyl) dithiocarbamate; lead N,N,N',N'-tetra-( $\gamma$ -( $\beta$ -phenanthryl)- $\Delta^2$ -n-pentenyl) dithiocarbamate; lead N,N,N',N'-tetra-( $\delta$ -( $\gamma$ -phenanthryl)- $\Delta^3$ -n-pentenyl) dithiocarbamate; and the like.

Moreover, our dithiocarbamate antioxidants comprise cycloaliphatic substituted compounds providing, for example, such compounds as lead N,N,N',N'-tetracyclopropyl dithiocarbamate; lead N,N,N',N'-tetra-( $\alpha$ -cyclobutyl)-amyl dithiocarbamate; lead N,N,N',N'-tetra-( $\beta$ -cyclobutyl)-isoamyl dithiocarbamate; and the like. Similarly, cycloaliphatic derivatives of the alkenyls can be substituted in the dithiocarbamate antioxidants of our invention providing compounds such as, for example, lead N,N,N',N'-tetra-( $\alpha$ -cycloheptyl)- $\Delta^1$ -propenyl dithiocarbamate; and the like.

Furthermore, R<sub>1</sub>, R<sub>2</sub>, R<sub>3</sub>, and R<sub>4</sub> can be different and be selected from hydrogen and organic radicals providing as dithiocarbamate antioxidants of our invention such compounds as, for example, lead N-methyl dithiocarbamate; lead N,N-diethyl dithiocarbamate; lead N,N-di-n-propyl dithiocarbamate; lead N-methyl, N-isopropyl

dithiocarbamate; lead N-n-butyl, N'-isoamyl dithiocarbamate; lead N,N,N'-triethenyl dithiocarbamate; lead N-ethyl, N-( $\Delta^1$ -propenyl), N'-( $\beta$ -phenyl)-n-propyl dithiocarbamate; lead N,N-di-sec-butyl, N'-( $\alpha$ -( $\alpha'$ -naphthyl)-n-propyl), N'-( $\alpha$ -cycloamyl)- $\Delta^2$ -propenyl dithiocarbamate; lead N-methyl, N-ethyl, N'-n-propyl, N'-n-butyl dithiocarbamate; and the like.

When X and X<sub>1</sub> of the aforementioned generic structure are oxygen, there is provided a general class of lead thiocarbamates. Thus, specific non-limiting examples of these compounds comprising the antioxidants of our invention include lead N,N,N',N'-tetra-methyl thiocarbamate; lead N,N,N',N'-tetra-ethenyl thiocarbamate; lead N,N,N',N'-tetra-(1-methyl- $\Delta^2$ -propenyl) thiocarbamate; lead N,N,N',N'-tetra-( $\alpha$ -phenylethyl) thiocarbamate; lead N,N,N',N'-tetra-( $\alpha$ -( $\alpha'$ -anthryl)- $\Delta^1$ -hexenyl) thiocarbamate; lead N,N,N',N'-tetra-cyclopropyl thiocarbamate; lead N,N,N',N'-tetra-( $\alpha$ -cycloheptyl)- $\Delta^1$ -propenyl thiocarbamate; lead N-methyl thiocarbamate; lead N,N-diethyl thiocarbamate; lead N,N'-di-n-propyl-thiocarbamate; lead N-methyl, N-isopropyl thiocarbamate; lead N-n-butyl, N'-isoamyl thiocarbamate; lead N,N,N'-triethenyl thiocarbamate; lead N-ethyl, N-( $\Delta^1$ -propenyl), N'-( $\beta$ -phenyl)-n-propyl thiocarbamate; lead N,N-di-sec-butyl, N'-( $\alpha$ -( $\alpha'$ -naphthyl)-n-propyl), N'-( $\alpha$ -cycloamyl)- $\Delta^2$ -propenyl thiocarbamate; lead N-methyl, N-ethyl, N'-n-propyl, N'-n-butyl thiocarbamate; and the like.

Referring to the aforementioned generic structure, when X is oxygen and X<sub>1</sub> is sulfur, there is provided a general class of mixed thio derivatives of lead carbamate comprising the antioxidants of our invention such as, for example, lead (N,N-diethyl-thio)-(N',N'-diethyl-dithio)-carbamate.

As shown above, R<sub>1</sub>, R<sub>2</sub>, R<sub>3</sub>, and R<sub>4</sub> can be the same or different and are selected from hydrogen or organic radicals. The selection of such radicals is contingent upon the solubility desired in the resulting compound. Thus, an antioxidant material for certain uses such as, for example, stabilizers for gasoline, diesel fuels, and lubricating oils, must exhibit relatively high solubility in hydrocarbons and an extremely low solubility in water to prevent extraction thereby. Likewise, a rubber antioxidant must possess certain compatibility and miscibility characteristics with the stock being protected. Similar considerations pertain for each class of substances for which our compounds are useful antioxidants.

In addition to our startling discovery that the aforementioned compounds provide effective oxygen stabilization, we have discovered that these compounds have the property of greatly increasing the effectiveness of previously known antioxidants of the arylamine type. Typical examples of these known arylamine antioxidants which are improved by employing therewith such sulfur-containing lead carbamates include N,N'-di-sec-butyl-p-phenylenediamine; N-n-butyl-p-aminophenol; N-isobutyl-p-aminophenol; N,N'-di- $\alpha$ -naphthyl-p-phenylenediamine; N,N'-di-isopropyl-p-phenylenediamine; N-phenyl- $\beta$ -naphthylamine; 4-aminodiphenylamine; 2-aminodiphenylamine; and the like. Thus, we have found that the sulfur-containing lead carbamates can be employed both as primary antioxidants and as synergists.

The compounds of our invention are further defined by reference to the following method of preparation which, while not restricting the scope of the variations possible in different embodiments of our invention, is representative of one method which we have employed in preparing the typical materials described herein. All quantities referred to herein are parts by weight.

#### LEAD N,N,N',N'-TETRA-n-BUTYL-DITHIOCARBAMATE

In a reaction vessel was placed 129 parts of di-n-butylamine and 400 parts of water. To the resulting solu-

tion was added 90 parts of carbon disulfide over a period of one hour, maintaining the reaction mixture at a temperature of approximately 15° C. The reaction mixture was then neutralized by adding thereto an approximately 10 normal sodium hydroxide solution using phenolphthalein as an indicator. The resulting solution was diluted to approximately 1,000 parts. One hundred parts of this solution was added to a solution of 19 parts of lead acetate and 100 parts of water. The resulting yellow curdy precipitate was filtered and dried. This crude lead N,N,N',N'-tetra-n-butyl dithiocarbamate was recrystallized from mixed hexanes, the resulting solid having a melting point of approximately 44 to 45° C. The product contained 33.46 per cent lead, while the empirical formula  $C_{18}H_{36}N_2S_4Pb$  requires 33.65 per cent lead.

The absorption of oxygen by hydrocarbon fuels can be measured directly by the standard method of the American Society of Testing Materials for determination of the oxidation stability of gasoline (Induction Period Method), ASTM designation: D525-46, as fully described in part III-A, ASTM Standards for 1946. According to this method the induction period is the period during which there is no drop in pressure, indicating no absorption of oxygen when the test material is placed in a testing bomb maintained at a temperature of 100° C. with an initial pressure of 100 pounds per square inch gauge of oxygen. The induction period increase (IPI) is the increase in the duration of this period caused by the addition of a protective substance, and is a direct measure of the protection afforded by such additive. Thus, the longer the IPI the more effective is the stabilizer. On the contrary, certain substances exert a pro-oxidant effect in which a negative IPI is obtained; that is, the duration of the induction period, or period of no absorption of oxygen, is less than in the absence of the additive.

As an example of the utility of sulfur-containing lead carbamates as primary antioxidants for various organic substances unstable to attack by oxygen, lead N,N,N',N'-tetra-n-butyl dithiocarbamate, also known as lead di-n-butyl dithiocarbamate, was prepared in accordance with the aforementioned procedure. To obtain the results shown herein alternately 3 milligrams and 6 milligrams of the additive were dissolved in 100 milliliters of a standard commercial gasoline, the properties of which are shown in Table I.

Table I

PHYSICAL AND CHEMICAL PROPERTIES OF A TYPICAL COMMERCIAL GASOLINE

| Test                    | Test Method                   | Results |
|-------------------------|-------------------------------|---------|
| Gum, mg./100 ml.:       |                               |         |
| Dissolved.....          | D381-50 <sup>1</sup>          | 1.8     |
| High Temp.....          | D381-50 <sup>1</sup>          | 1.8     |
| Copper Dish.....        | U. O. P. H-11-43 <sup>2</sup> | 31.4    |
| Induction Period.....   | D525-49 <sup>1</sup>          | 230.0   |
| Sulfur, percent.....    | D90-50T <sup>1</sup>          | 0.076   |
| Acid Heat.....          | D481 <sup>2</sup>             | 81.0    |
| Bromine Number.....     | DI158-51T <sup>1</sup>        | 43.9    |
| Specific Gravity.....   | D287-39 <sup>1</sup>          | 64.2    |
| Distillation Range..... | D86-46 <sup>1</sup>           |         |

| Percent evaporated | ° F. |
|--------------------|------|
| Initial.....       | 92   |
| 10.....            | 128  |
| 50.....            | 215  |
| 90.....            | 381  |
| Final.....         | 410  |

<sup>1</sup> Fully described in "Petroleum Products and Lubricants," ASTM Standards for 1951.

<sup>2</sup> U. O. P. Laboratory Test Methods for Petroleum and Its Products, 1940.

<sup>3</sup> Fully described in "Petroleum Products and Lubricants," ASTM Standards prior to 1949.

Typical of the results obtained using the aforementioned Induction Period Method, 3 milligrams of lead di-

n-butyl dithiocarbamate per 100 milliliters of gasoline produced an IPI of 125 minutes, and 6 milligrams produced an IPI of 145 minutes. With another commercial gasoline of similar physical and chemical properties and having an Induction Period of 240 minutes, 3 milligrams of lead di-n-butyl dithiocarbamate per 100 milliliters of gasoline produced an IPI of 100 minutes, and 6 milligrams produced an IPI of 115 minutes. Similar results are obtained when other typical compounds of our invention are employed in concentrations of 3 milligrams and 6 milligrams per 100 milliliters of gasoline. Thus, for example, 3 milligrams of lead N,N,N',N'-tetra-sec-butyl dithiocarbamate produced an IPI of 105 minutes, and 6 milligrams produced an IPI of 130 minutes; 3 milligrams of lead N,N,N',N'-tetra-n-propyl dithiocarbamate produced an IPI of 120 minutes, and 6 milligrams produced an IPI of 135 minutes; 3 milligrams of lead N,N,N',N'-tetramethyl dithiocarbamate produced an IPI of 130 minutes, and 6 milligrams produced an IPI of 155 minutes; 3 milligrams of lead N,N,N',N'-tetraethyl dithiocarbamate produced an IPI of 110 minutes, and 6 milligrams produced an IPI of 130 minutes; 3 milligrams of lead N,N,N',N'-tetraisopropyl dithiocarbamate produced an IPI of 115 minutes, and 6 milligrams produced an IPI of 140 minutes; 3 milligrams of lead N,N,N',N'-tetraisobutyl dithiocarbamate produced an IPI of 135 minutes, and 6 milligrams produced an IPI of 150 minutes; and 3 milligrams of lead N,N,N',N'-tetra-n-amyl dithiocarbamate produced an IPI of 130 minutes, and 6 milligrams produced an IPI of 150 minutes.

The compounds of our invention likewise provide protection to rubber stocks and the like. This can be determined by measuring the degree to which a test piece so compounded retains its elasticity after being subjected to accelerated aging according to the procedure of ASTM designation: D572-42 for a period of 96 hours at a temperature of 70° C. in the presence of oxygen pressure initially at 300 pounds per square inch gauge. By determining both the tensile strength and the ultimate elongation of such test pieces, it is found that our compounds greatly improve these properties of such rubber stocks.

As an example of the utility of our compounds currently providing both antioxidant activity and imparting a synergistic effect to antioxidants of the arylamine type, 3 milligrams of lead N,N,N',N'-tetra-n-butyl dithiocarbamate and 3 milligrams of N,N'-di-sec-butyl-p-phenylenediamine were dissolved in 100 milliliters of a standard commercial gasoline having physical and chemical properties similar to those shown in Table I and having an Induction Period of 225. Alternately, 1.5 milligrams of lead di-n-butyl dithiocarbamate and 1.5 milligrams of N,N'-di-sec-butyl-p-phenylenediamine were dissolved in 100 milliliters of a standard commercial gasoline. The results of these tests are shown in Table II.

Table II  
EFFECT ON INDUCTION PERIOD INCREASE OF GASOLINES

| Total Concentration of Mixture, mg./100 ml. | Induction Period Increase, Minutes |                |                                       |                       |
|---------------------------------------------|------------------------------------|----------------|---------------------------------------|-----------------------|
|                                             | From Mixture                       | From Arylamine | From Sulfur-Containing Lead Carbamate | Net Gain From Mixture |
| 60                                          |                                    |                |                                       |                       |
| 65                                          |                                    |                |                                       |                       |
| 66                                          | 6.....                             | 505            | 180                                   | 125                   |
| 66                                          | 6.....                             | 505            | 180                                   | 100                   |
| 66                                          | 3.....                             | 310            | 100                                   | 120                   |
|                                             |                                    |                |                                       | 90                    |

Similar results are obtained by the use of other species of our invention in combination with other arylamine antioxidants, as, for example, such mixtures as lead N,N,N',N'-tetra-isobutyl dithiocarbamate and N-n-butyl-p-aminophenol; lead N,N,N',N'-tetra-isobutyl dithiocarbamate and N,N'-di-sec-butyl-p-phenylenediamine;

tetra-isobutyl thiocarbamate and N,N'-di-isopropyl-p-phenylenediamine; lead N,N,N',N'-tetra-isobutyl thiocarbamate and N-phenyl- $\beta$ -naphthylamine; lead N,N,N',N'-tetra-isobutyl thiocarbamate and 4-aminodi-phenylamine; lead N,N,N',N'-tetra-isobutyl thiocarbamate and 2-aminodiphenylamine; lead N,N,N',N'-tetra-t-butyl thiocarbamate and N-n-butyl-p-aminophenol; lead N,N,N',N'-tetra-t-butyl thiocarbamate and N,N'-di-sec-butyl-p-phenylenediamine; lead N,N,N',N'-tetra-t-butyl thiocarbamate and N-isobutyl-p-aminophenol; lead N,N,N',N'-tetra-t-butyl thiocarbamate and N,N'-di- $\alpha$ -naphthyl-p-phenylenediamine; lead N,N,N',N'-tetra-t-butyl thiocarbamate and N,N'-di-isopropyl-p-phenylene-diamine; lead N,N,N',N'-tetra-t-butyl thiocarbamate and N-phenyl- $\beta$ -naphthylamine; lead N,N,N',N'-tetra-t-butyl thiocarbamate and 4-aminodiphenylamine; lead N,N,N',N'-tetra-t-butyl thiocarbamate and 2-aminodi-phenylamine; lead N,N,N',N'-tetra-sec-butyl thiocarbamate and N-n-butyl-p-aminophenol; lead N,N,N',N'-tetra-sec-butyl thiocarbamate and N,N'-di-sec-butyl-p-phenylenediamine; lead N,N,N',N'-tetra-sec-butyl thiocarbamate and N-isobutyl-p-aminophenol; lead N,N,N',N'-tetra-sec-butyl thiocarbamate and N,N'-di- $\alpha$ -naphthyl-p-phenylenediamine; lead N,N,N',N'-tetra-sec-butyl thiocarbamate and N,N'-di-isopropyl-p-phenylenediamine; lead N,N,N',N'-tetra-sec-butyl thiocarbamate and N-phenyl- $\beta$ -naphthylamine; lead N,N,N',N'-tetra-sec-butyl thiocarbamate and 4-aminodiphenylamine; lead N,N,N',N'-tetra-sec-butyl thiocarbamate and 2-aminodiphenylamine; lead N,N,N',N'-tetraethyl thiocarbamate and N-n-butyl-p-aminophenol; lead N,N,N',N'-tetraethyl thiocarbamate and N,N'-di-sec-butyl-p-phenylenediamine; lead N,N,N',N'-tetraethyl thiocarbamate and N-isobutyl-p-aminophenol; lead N,N,N',N'-tetraethyl thiocarbamate and N,N'-di- $\alpha$ -naphthyl-p-phenylenediamine; lead N,N,N',N'-tetraethyl thiocarbamate and N,N'-di-isopropyl-p-phenylenediamine; lead N,N,N',N'-tetraethyl thiocarbamate and N-phenyl- $\alpha$ -naphthylamine; lead N,N,N',N'-tetraethyl thiocarbamate and 4-aminodi-phenylamine; lead N,N,N',N'-tetraethyl thiocarbamate and 2-aminodiphenyl-amine; lead N,N,N',N'-tetra-n-amyl thiocarbamate and N-n-butyl-p-aminophenol; lead N,N,N',N'-tetra-n-amyl thiocarbamate and N,N'-di-sec-butyl-p-phenylenediamine; lead N,N,N',N'-tetra-n-amyl thiocarbamate and N-isobutyl-p-aminophenol; lead N,N,N',N'-tetra-n-amyl thiocarbamate and N,N'-di- $\alpha$ -naphthyl-p-phenylenediamine; and the like.

Mixtures of the sulfur-containing lead carbamates of our invention when employed along with known arylamine 50 antioxidants likewise provide protection to rubber stocks and the like. This can be determined by measuring the degree to which a test piece so compounded retains its elasticity after being subjected to accelerated aging according to the above described procedure. By determining 55 both the tensile strength and ultimate elongation of such test pieces, it is found that our antioxidant-synergist compositions greatly improve the functioning of aryl antioxidants and overcome some of their inherent disadvantages such as migration and bleeding.

60 The quantities of the compounds of our invention incorporated in the materials to be stabilized are not critical and depend largely upon the type of material being stabilized and the conditions under which the exposure to oxygen occurs. For example, with gasolines, diesel fuels, 65 mineral oils, and similar materials, the compounds of our invention are preferably employed in concentrations between the limits of approximately 0.1 and 15 milligrams per 100 milliliters of material to be stabilized. For other materials, such as, for example, soaps and natural and 70 synthetic elastomers, somewhat larger amounts of the stabilizers of our invention are preferred and can be tolerated. Thus, in such materials we employ between approximately 0.1 and 2 parts of antioxidant per 100 parts of oxidizable material. Thus, our compounds can be satisfactorily employed in a wide range of concentrations, 75

and we do not intend that our invention be restricted to the specific quantities mentioned herein.

We have disclosed a number of preferred embodiments of our invention and illustrated several means whereby protection can be afforded to organic materials sensitive to attack by oxygen. Our invention is not intended to be limited to the specific embodiments herein or to the means described herein for obtaining the advantages possible in employing our compounds, as other methods of practicing our invention will be apparent to those skilled in the art.

We claim:

1. A new composition stable to oxidation and consisting essentially of gasoline normally tending to deteriorate in the presence of oxygen and containing a synergistic antioxidant composition consisting essentially of substantially equal amounts by weight N,N'-di-sec-butyl-p-phenylene diamine and lead N,N,N',N'-tetra-n-butyl dithiocarbamate, each being present within the range of 0.1 to 15 milligrams per 100 milliliters of said gasoline.

2. Gasoline normally tending to deteriorate in the presence of oxygen and containing a synergistic antioxidant combination of N,N'-di-sec-butyl-p-phenylene di-

amine and lead N,N,N',N'-tetra-n-butyl dithiocarbamate, said phenylene diamine and said dithiocarbamate each being present in said gasoline in an amount within the range of 0.1 to 15 milligrams per 100 milliliters of said gasoline.

3. Gasoline normally tending to deteriorate in the presence of oxygen containing N,N'-di-sec-butyl-p-phenylenediamine and lead N,N,N',N'-tetra-n-butyl-dithiocarbamate, said phenylenediamine and said dithiocarbamate each being present in said gasoline in amount equivalent to 3 mg./100 ml. of said gasoline.

5

10

15

20

#### UNITED STATES PATENTS

##### References Cited in the file of this patent

|           |                |       |               |
|-----------|----------------|-------|---------------|
| 2,016,648 | Orelup         | ----- | Oct. 8, 1935  |
| 2,160,851 | Faust          | ----- | June 6, 1939  |
| 2,356,661 | Dawning et al. | ----- | Aug. 22, 1944 |
| 2,363,012 | Miller et al.  | ----- | Nov. 21, 1944 |
| 2,382,781 | Dawning et al. | ----- | Aug. 14, 1945 |
| 2,395,382 | Walters        | ----- | Feb. 19, 1946 |
| 2,400,106 | Denison et al. | ----- | May 14, 1946  |
| 2,614,987 | Dreher et al.  | ----- | Oct. 21, 1952 |